

## UNITED STATES PATENT OFFICE

2,164,280

## PHOTOGRAPHIC DEVELOPER

Edmund W. Lowe, Chicago, Ill., assignor to The Edwal Laboratories, Inc., Chicago, Ill., a corporation of Illinois

No Drawing. Application September 20, 1937,  
Serial No. 164,703

12 Claims. (Cl. 95—88)

My invention relates to the art of photography and particularly to the development of photographic emulsions to produce fine-grained or even-grained images.

For a number of years, there has been considerable interest in the production of so-called fine-grained images, and developing compositions adapted for producing fine-grained or even-grained images have come to be known as "fine grain developers." The increased interest in fine grain developers is due to a considerable extent to the increased use of cameras employing negatives of such a small size that the print is made by projecting the film image onto the photographic paper instead of printing by direct contact. Conversely, improvements in films and improvements in fine grain developers have made possible the increased use of miniature cameras, so that the production of improved fine-grain developers cannot be said to be merely in response to the demand for the production of images of the fine-grained or even-grained type.

So called coarse-grained images, I have determined, result very largely, if not entirely, from a clumping up of silver particles during development, with the result that the particles, instead of being evenly distributed throughout the emulsion, are found in patches or clumps distinctly discernible under a microscope. The result is that, if a negative developed in the ordinary way so as to produce a coarse grain is enlarged only very slightly, the print has a mottled and uneven appearance. Even some of the so-called fine-grain developers will show a certain amount of graininess if a degree of enlargement be attempted appreciably in excess of 4 or 5 diameters, although some fairly satisfactory fine-grain negatives have been produced by some of the fine-grained developers which can be enlarged to approximately 20 diameters without appreciable development of a mottled or grainy appearance.

Some fine-grain developers have also been suggested which produce negatives capable of enlargement in excess of 20 to 25 diameters, indeed up to 50 or 60 diameters, without appreciable graininess in the enlargement. All of these developers with which I am familiar, however, have certain disadvantages. The marked disadvantage of one type of fine-grain developer is that the negatives produced tend to be rather flat and the films must be exposed to light while in the camera fifty to one hundred percent longer in order to obtain sufficient density in the negative. Other fine-grain developers capable of very great enlargement without the development of graini-

ness have the disadvantage that the negatives developed in them tend to have blocked-up highlights unless the developing time be very carefully regulated. Another disadvantage found in substantially all fine-grain developers produced heretofore is that they tend to produce a coarser grain than otherwise if the negative has been overexposed. They also have the disadvantage that, while the negatives are capable of very great enlargement without the appearance of grain, the enlarged images tend to lack critical definition, and the very large pictures produced do not faithfully record the surface texture of objects photographed.

It is the object of my present invention to develop fine-grained images in a more satisfactory manner than has been done heretofore.

A further object is to provide an improved fine-grain developer which produces very fine, even-grained images without the disadvantages inherent in negatives produced by previously known fine-grain developers.

In general, I accomplish the objects of my invention by the use of primary and secondary developing agents of a character to be defined hereinbelow, a substance capable of forming soluble, substantially stable complexes with the silver salts of the emulsion, and a soluble sulphite salt of a relatively strong base, the developing solution as a whole having a pH of 7 to 7.8 and particularly in certain preferred embodiments from 7.3 to 7.5. The foregoing general identification of the developer of my invention is, of course, to be understood in the light of the more particular consideration of the ingredients as discussed hereinbelow. In general, it may be stated, however, that I may, under certain circumstances, dispense with the use of the secondary developing agent, in which case somewhat modified results are obtained.

The primary developing agent which I employ is p-methylaminophenol or one of its salts, such as the sulphate commonly known as "metol." (The terms "elon", "rhodol" and "pictol" are employed in the trade to identify the same compound.) I may also employ p-methylaminocresol, with the methyl group of the cresol in either of the two possible positions, but, in general, I prefer the use of the metol type of compound. If a relatively soft image negative is desired, no other developing agent is necessary. If, however, stronger contrast is desired, a secondary developing agent may be used, this secondary developing agent being one having a relatively low reduction potential. The second developing agent

is preferably p-hydroxyphenylglycine, commonly known as "glycin." Other developing agents of relatively low potential may be employed, however, such as chlorohydroquinone, bromohydroquinone, or p-aminophenol and its salts.

In the fine-grain developer of my present invention, I do not employ any alkaline accelerators such as carbonates, borates, etc. A sulphite such as sodium sulphite is employed, however, which shows a mild alkaline reaction in solution, and the proportion of the sulphite can be so regulated as to produce the desired pH in the solution of the final composition. I may employ any soluble sulphite of an alkali or alkali earth metal or a soluble sulphite of an organic base. Preferably, I use sodium sulphite in amounts to introduce 50 to 150 grams of sodium sulphite per liter of water. Ammonium chloride is the preferred substance of the group defined as substances capable of forming substantially stable complexes with silver salts, but ammonium salts of relatively strong acids having a pH in solution of less than 6 will function satisfactorily as well as certain amine salts and sodium thiosulphate. The latter compound, however, must be used with very great care and in very small proportions, and those proportions must be properly balanced with respect to the other chemical or desirable results will not be obtained.

Before referring to specific examples, I wish to point out that the primary developing agent which I employ is one which is sufficiently energetic to produce a satisfactory image in a reasonable length of time when the pH of the developing solution lies between 7 and 7.8. Moreover, the primary developing agent which I employ is and must be "soft-working", that is, used alone, it must not produce negatives of high contrast unless the developing time is unduly prolonged. The primary developing agents identified hereinabove have these properties. Obviously, therefore, if a relatively soft negative image is desired, the secondary developing agent need not be employed. The secondary developing agent, however, as described a developing agent of relatively low production potential, results in the development of an image with strong contrast without affecting the fine grain of the image deleteriously.

The following examples illustrate compositions for producing fine-grained images on photographic negatives, all of these examples coming within the scope of the general description of my invention contained hereinabove.

#### 55 Example 1

|                              |       |     |
|------------------------------|-------|-----|
| Distilled water              | liter | 1   |
| p-Methylaminophenol sulphate | grams | 8   |
| p-Hydroxyphenylglycine       | do    | 8   |
| Sodium sulphite              | do    | 100 |
| Ammonium chloride            | do    | 5   |

The pH of this solution is 7.4.

#### 60 Example 2

|                              |       |     |
|------------------------------|-------|-----|
| Distilled water              | liter | 1   |
| p-Methylaminophenol sulphate | grams | 8   |
| p-Hydroxyphenylglycine       | do    | 5   |
| Sodium sulphite              | do    | 100 |
| Ammonium chloride            | do    | 5   |

#### 65 Example 3

|                              |       |     |
|------------------------------|-------|-----|
| Distilled water              | liter | 1   |
| p-Methylaminophenol sulphate | grams | 8   |
| p-Hydroxyphenylglycine       | do    | 2   |
| Sodium sulphite              | do    | 100 |
| Ammonium chloride            | do    | 5   |

#### Example 4

|                              |       |     |
|------------------------------|-------|-----|
| Distilled water              | liter | 1   |
| p-Methylaminophenol sulphate | grams | 8   |
| p-Hydroxyphenylglycine       | do    | 8   |
| Sodium sulphite              | do    | 100 |
| Sodium thiosulphate          | do    | 0.5 |

#### Example 5

|                                   |       |     |
|-----------------------------------|-------|-----|
| Water                             | liter | 1   |
| p-Methylaminophenol hydrochloride | grams | 8   |
| Chlorohydroquinone                | do    | 5   |
| Sodium sulphite                   | do    | 120 |
| Ammonium chloride                 | do    | 10  |

#### Example 6

|                              |       |    |
|------------------------------|-------|----|
| Water                        | liter | 1  |
| p-Methylaminophenol sulphate | grams | 2  |
| p-Hydroxyphenylglycine       | do    | 1  |
| Sodium sulphite              | do    | 90 |
| Ammonium chloride            | do    | 10 |

The pH of the solutions given in the examples hereinabove is, in each case, between 7 and 7.8, and, for the most part, fairly close to 7.4. While the examples are given as indicating water solutions, it is to be understood that the common way of marketing my developer is to sell it as a dry mixture, and so proportion the ingredients that, when a given quantity of the mixture as a whole is dissolved in a given quantity of water, a suitable developing solution will be produced. It is to be noted that Examples 1 to 5, inclusive, show solutions which are suitable for developing several rolls of film. Example 6, however, illustrates a formula good for developing only a single roll of film, and the solution can then be discarded as worthless. I may also prepare stock solutions of my developer which can be diluted down to the desired strength, although, when employing my preferred group of ingredients and producing a solution capable of developing several rolls of film, the total amount of material in solution is such that a stock solution cannot be produced which is capable of dilution to such an extent as to warrant its use under ordinary circumstances.

It will be noted that Examples 1 to 3, inclusive, show decreasing proportions of the secondary developing agent, in this case p-hydroxyphenylglycine. Example 1 can be employed to produce relatively sharp images, and the amount of contrast obtainable decreases from Example 1 through Example 3, the latter producing images with considerably less contrast than Example 1. By leaving out the secondary developing agent entirely, the amount of contrast can be still further decreased.

Each of the examples given above employs a substance capable of forming a fairly stable water soluble complex with silver bromide, in all cases except one ammonium chloride being the ingredient in question, the other case being Example 4 where sodium thiosulphate is substituted. As stated previously, the proportion of sodium thiosulphate employed is apt to be very critical and, in the example given, if more than half a gram of sodium thiosulphate be employed, there will be a strong probability if not a certainty of getting a foggy image as a result. For this reason, I prefer to employ ammonium chloride or other ammonium salt. It is not absolutely necessary, however, that ammonium chloride or a similar agent be used, although much more dependable results are obtained by its use. Should those skilled in the art wish, for any reason, to avoid the use of ammonium chloride, they may in part

make up for its loss by increasing somewhat the amount of sodium sulphite used. The sodium sulphite in the fine-grain developer of my present invention has a three-fold function. In the first place, it has a buffer action. Secondly, it exerts a solvent action on silver bromide and this accounts for the fact that to some extent the chloride may be compensated for by increasing the proportion of sulphite. Thirdly, the sodium sulphite has a preserving action, it being well known that it has been employed primarily as a preservative in many commercial developers used in the past. With respect to the solvent action of sodium sulphite, it is to be noted that, in general, it tends to form soluble complexes with silver bromide, but these soluble complexes are not sufficiently stable to prevent precipitation of silver bromide out of solution under certain conditions. Indeed, the complex molecules formed with ammonium chloride and silver bromide are not entirely stable but they are appreciably more stable than the soluble complexes including sodium sulphite and are adequately stable to produce the results desired. Accordingly, when I refer to the production of substantially stable complexes with silver bromide, this expression may be interpreted as meaning more stable than the complexes formed by the use of sodium sulphite.

In general, I may secure the objects of my invention if I employ ingredients selected from the groups or classes discussed hereinabove, and control the proportion of ingredients so that the pH of the developing solution is somewhere between 7 and 7.8. I find, however, that in general the advantages of my invention are more marked if the pH of the developing solution is between 7.3 and 7.5, particularly when the preferred ingredients are employed, namely, the specific ingredients given in Example 1. As noted with respect to this particular example, the pH is 7.4. This particular formula may be modified slightly, however, to bring the pH down slightly below 7.4, say 7.34, and for some purposes somewhat improved results even can be obtained than with the specific formula of Example 1. It is to be noted that all of the ingredients given in Example 1, with the exception of the sodium sulphite, possess an acid reaction in solution. Sodium sulphite is a mild alkali, a 10% solution of sodium sulphite having a pH of only 9.7. Indeed, in ordinary photographic work, sodium sulphite is never considered an alkali, so that in the parlance of the industry, the developer of my invention does not use an alkali. Nevertheless, by the buffer action of the sodium sulphite, the pH of the solution as a whole may be controlled, and the proportion of sodium sulphite may be modified for this purpose. With respect to modifying the proportions of ingredients given in Example 1, it may be stated that the "metol" may be present in the final solution (the solution being based on the use of one liter of water) in proportions of 1 to 20 grams, the glycine in proportions of from 1 to 15 grams, the sodium sulphite in proportions of from 50 to 150 grams, and the ammonium chloride in proportions up to approximately 30 grams. Whatever the proportions may be, the ingredients may be balanced so that the pH of the final solution is within the broad range defined, but preferably within the specific range discussed hereinabove, namely from 7.3 to 7.5.

The developing characteristics of my improved fine-grain developer are such that in general somewhat longer time may be required than is

normally required when employing so-called fine-grain developers marketed before my invention. For the further understanding of those skilled in the art, I give below the approximate developing time for different types of films based upon the use of a developer substantially identical in proportions of ingredients and strength of solution given in Example 1.

|                                                                                  | Minutes  |
|----------------------------------------------------------------------------------|----------|
| (1) For fine-grain panchromatic films such as du Pont's Micropan or Agfa Finopan | 10       |
| (2) For most ordinary emulsions of both the panchromatic and orthochromatic type | 7 to 10  |
| (3) For slow developing films such as Selo hypersensitive panchromatic           | 16 to 20 |
|                                                                                  | 15       |
|                                                                                  | 25 to 30 |

The outline of developing time given above is not meant to be exhaustive but only sufficiently representative so that those skilled in the art will in general be able to gauge developing time for any particular kind of film from this general outline. It is a characteristic of this developer that when several rolls of film are developed in the same solution, the development time must be increased somewhat for each successive roll in order to obtain the same contrast.

The improved developers of my invention produce negatives having exceedingly fine, even grain, so that enlargements up to 50 diameters and more can be made from them without difficulty. Furthermore, the big enlargements from such negatives reproduce the outline of the original accurately, and the surface texture of the subject photographed is reproduced with much greater fidelity than enlargements from negatives processed from older types of so-called fine-grain developers. It is a marked characteristic of my new developing solutions that the negatives developed by their use do not readily lose detail or block up in the regions of highlight, as is usually found to be the case in older types of fine-grain developers. The developer of my invention, whether in the dry form or in solution, keeps well, does not stain the hands or clothing in the normal course of photographic processing, and generally, from a practical standpoint, is very satisfactory in those properties which are not so directly concerned with the finished negative.

Additional advantages and important characteristics of the developers of my invention have to do with the time element both from the standpoint of developing time and exposure time of the film in the camera. Some developers tend to show extreme variations in the quality of the negative when there is an appreciable variation in the developing time. However, when the developer of my invention is employed, there may be quite a considerable variation in the developing time and this does not cause extreme variations in the quality of the negative providing reasonable care otherwise is used. The second important characteristic is that negatives which have been subjected to considerable over-exposure, and hence possess a high density, do not tend to have a coarse grain when developed by the use of my invention, whereas similar negatives, processed in previous developers, especially certain ones of the previously employed fine-grain developers, show marked coarseness of grain, notwithstanding the fact that the same developer used on a negative exposed for a normal period of time would not produce a coarse grained

negative. Indeed, negatives may be exposed up to ten times the normal amount for given conditions, and the negative so exposed can be developed by means of my developer without the production of coarse grain. Needless to say, over-exposure of such duration is not recommended, but the fact that such an over-exposed negative may be developed and a fine-grain image produced by my developer, illustrates the point that a more than normal exposure of the film may be had so as to produce a relatively heavy image. Since detail is not lost in regions of highlight when employing my developer, and, therefore, blocking out is not a factor to be reckoned with, the relatively heavy image will contain enough silver so as to record detail very sharply even on very big enlargements. This opens up possibilities in photography not heretofore present in the miniature field. Indeed, relatively big enlargements may be made from films which have all of the appearance of contact prints made from relatively very much larger films, and the surface texture of such substances as sand, snow, skin, cloth, trees, grass and the like is reproduced so faithfully that results can be obtained in no sense obtainable with other developers with which I am familiar.

I have described my invention in relatively great detail for the benefit of those skilled in the art but it is understood that the scope of my invention is limited only by the definitions thereof contained in the appended claims.

What I claim as new and desire to protect by Letters Patent of the United States is:

35 1. A fine grain photographic developer comprising a developing agent of a class consisting of paramethylaminophenol, paramethylaminocresols, and their salts, an ammonium salt of a relatively strong acid, and a soluble sulphite, the proportions of ingredients being balanced so that the developer in solution has a pH of 7 to 7.8.

2. A fine grain photographic developer comprising a developing agent of a class consisting of paramethylaminophenol, paramethylaminocresols, and their salts, an ammonium salt of a relatively strong acid, and a sodium sulphite, the proportions of ingredients being balanced so that the developer in solution has a pH of 7 to 7.8.

3. A fine grain photographic developer comprising as a main developing agent paramethylaminophenol or one of its salts, a secondary developing agent of relatively low reduction potential capable of functioning in substantially neutral solutions, an ammonium salt of a relatively strong acid, and a soluble sulphite, the proportions of ingredients being such that the developer in solution has a pH of 7 to 7.8.

4. A fine grain photographic developer comprising as a main developing agent paramethylaminophenol or one of its salts, a secondary developing agent of relatively low reduction potential capable of functioning in substantially

neutral solutions, ammonium chloride, and a soluble sulphite, the proportions of ingredients being such that the developer in solution has a pH of 7 to 7.8.

5. A fine grain photographic developer comprising as a main developing agent paramethylaminophenol or one of its salts, parahydroxyphenylglycine, ammonium chloride, and a soluble sulphite, the proportions of ingredients being such that the developer in solution has a pH of 7 to 7.8. 10

6. A fine grain photographic developer comprising as a main developing agent paramethylaminophenol or one of its salts, a secondary developing agent of relatively low reduction potential capable of functioning in substantially neutral solutions, ammonium chloride, and sodium sulphite, the proportions of ingredients being such that the developer in solution has a pH of 7 to 7.8. 15

7. A fine grain photographic developer comprising p-methylaminophenolsulphate, 1 to 20 parts; p-hydroxyphenylglycine, 1 to 15 parts; sodium sulphite, 50 to 150 parts; and ammonium chloride, 1 to 30 parts, said developer having a pH of 7 to 7.8, and possessing the property of producing extremely fine grain images with sharp outlines and ample detail in the highlights. 20

8. A fine grain photographic developer comprising as a primary developing agent p-methylaminophenol or one of its salts, a secondary developing agent of relatively low reduction potential, a soluble ammonium salt having a pH in solution lower than 7, and a sufficient amount of a soluble sulfite having a pH in solution greater than 7 to produce a developing composition which in solution has a pH of 7.3 to 7.5. 30

9. A fine grain photographic developer comprising p-methylaminophenol, p-hydroxyphenylglycine, ammonium chloride and sodium sulphite, said developer in solution having a pH of 7.3 to 7.5. 40

10. A fine grain developer, comprising substantially equal proportions of p-methylamino phenol sulphate, and p-hydroxyphenylglycine, a somewhat lesser proportion of ammonium chloride, and enough sodium sulphite to cause the developer as a whole, in solution, to have a pH of between 7.0 and 7.8. 45

11. A fine grain developer comprising "metol" as a primary developing agent, up to substantially equal proportions of a secondary developing agent of low potential, ammonium chloride, and enough sodium sulphite to cause the developer as a whole, in solution, to have a pH of about 7.4. 50

12. A fine grain developer comprising the following ingredients in the proportions called for: "metol", about 8 grams; "glycine", about 8 grams; ammonium chloride, about 5 grams; and sodium sulphite, about 100 grams; said developer adapted to be dissolved in water to produce a solution having a pH of approximately 7.4. 55 60

EDMUND W. LOWE.